

No. 890,230.

PATENTED JUNE 9, 1908.

J. T. JONES.

METHOD OF DEPHOSPHORIZING ORES.

APPLICATION FILED DEC. 23, 1907.



Witnesses:

Paul Payford.  
Cas H. Buell.

Inventor:

John T. Jones.  
By Dyerforth, Lee, Chittenden & Miles,  
Atty's.

# UNITED STATES PATENT OFFICE.

JOHN T. JONES, OF IRON MOUNTAIN, MICHIGAN, ASSIGNOR OF ONE-HALF TO GEORGE A. ST. CLAIR, OF DULUTH, MINNESOTA.

## METHOD OF DEPHOSPHORIZING ORES.

No. 890,230.

Specification of Letters Patent.

Patented June 9, 1908.

Application filed December 23, 1897. Serial No. 407,769.

To all whom it may concern:

Be it known that I, JOHN T. JONES, a citizen of the United States, residing at Iron Mountain, in the county of Dickinson and State of Michigan, have invented a new and useful Method of Dephosphorizing Ores, of which the following is a specification.

My invention relates to an improved method of treating ores to effect dephosphorizing thereof, and more especially iron and manganese ores, in either finely divided or lump form.

My invention is based upon the following facts: first, that when iron or manganese are subjected, for a time sufficiently prolonged and while under confinement against access thereto of oxygen, to the action of a hot reducing gas, and raised thereby to a temperature which will render the metal constituent sufficiently plastic, without however fusing the silicious constituents, the oxid particles are reduced to metal and caused to agglomerate forming what may be characterized as "sponge." Second, that as the temperature to which the ore is required to be subjected for the above purpose does not reach that necessary to bind phosphorus to the metal, volatiles freed from hydrocarbon fuel by the decomposition thereof and passed through the ore undergoing reduction will readily combine with any phosphoric acid in the ore and carry it off.

My object is to provide an improved method of procedure which, while taking advantage of the facts above set forth, will effect dephosphorization and reduction of the ore in one continuous operation and in a manner both effective and economical.

In the accompanying drawing I show, for purpose of illustration by a view mainly in sectional elevation, an ore-reducing furnace adapted for practicing my method in one approved way; sufficient of the structure only being shown to render intelligible the description of the operation.

A stack 1 of suitable height and dimensions is kept filled through its top with the ore to be treated. If the ore is in a finely divided condition, lumps of coke or other refractory material may be charged into the stack with the ore to render the mass suitably interstitial or porous for the ready passage through it of the reducing gases. These gases are generated in a suitable furnace 2 and discharged therefrom, under force

from one or more twayers 3 through a passage 4 into the lower part of the stack. No appreciable amount of air is admitted to the stack below the openings 5, the opening 6 shown through which the reduced ore is withdrawn, being provided with a suitable closing means (not shown).

The hot reducing gas, or gases, entering through the passage 4 rises through the column of ore confined in the stack, the temperature and volume of the gas, and the withdrawal of ore at 6, being so regulated in practice that by the time the ore descends past the passage 4 all its oxid constituents will have been heated to a deoxidizing temperature and thoroughly reduced to metal. The ports 5, which are located above the reducing zone, admit air to permit combustion of the more or less spent gases rising thereto for the purpose of pre-heating the air in the top of the stack.

Above the passage 4 and preferably in a plane near which reduction of the ore reaches completion, are one or a plurality of inlets 7 through which hydrocarbon fuel is forced or injected into the mass of ore. At the inlets I show coal-hoppers 8 discharging into cylinders 9 fitted with, preferably, hydraulic rams 10. The hoppers 8 may be provided with hinged covers 11, or the like, to exclude air. The object of this construction is to provide a means whereby carbonaceous fuel, as for example bituminous coal, may be forced in suitable quantity into the hot mass of ore. If it is desired to employ a liquid hydrocarbon, suitable injectors may be substituted for the coal rams. The heat of the mass into which this fuel is forced decomposes the fuel causing its hot volatile constituent to mingle with the gases rising from the passage 4 and ascend therewith through the ore.

It is to be understood that the heat to which the ore is subjected at and above the inlets 7, while sufficient to reduce the metallic oxides and cause agglomeration of the metal particles, is insufficient to bind phosphorus to the metal. Therefore the volatile products of decomposition of the fresh fuel, which have great affinity for phosphoric acid, will collect or at least greatly aid in collecting and carrying off all or most of the phosphorus content of the ore.

What I claim as new, and desire to secure by Letters Patent, is—

1. The method of dephosphorizing ore,

which consists in subjecting a mass thereof under confinement to the action of reducing gas, at a reducing temperature insufficient to bind phosphorus to the metal, and introducing into the mass, while being thus subjected, 5 fresh hydrocarbon fuel.

2. The method of deporphorizing ore, which consists in subjecting a mass thereof under confinement to the action of reducing 10 gas, at a reducing temperature insufficient to bind phosphorus to the metal and forcing coal into the mass while it is being thus subjected.

3. The method of deporphorizing ore

which consists in subjecting a confined and 1 slowly descending column thereof to the reducing action of reducing gas introduced into the lower part of the column, the temperature of the gas being insufficient to bind phosphorus to the metal, and forcing into the 20 descending column at a point near which reduction reaches completion, fresh hydrocarbon fuel.

JOHN T. JONES.

In presence of—

A. U. THORIEN,  
R. A. SCHAEFER.